

Dec. 17, 1935.

M. G. SNELLING

2,024,257

TREATMENT OF WOOD

Filed Jan. 27, 1934



Fig. 1



Fig. 2



Fig. 3



Fig. 4

Marjorie G. Snelling

INVENTOR

BY W. O. Snelling,

ATTORNEY

## UNITED STATES PATENT OFFICE

2,024,257

## TREATMENT OF WOOD

Marjorie G. Snelling, Allentown, Pa.

Application January 27, 1934, Serial No. 708,579

10 Claims. (Cl. 99—12)

My invention relates to improvements in methods of treating wood and more particularly relates to improved means of surfacing or finishing wood for use in cabinet making or for any other purpose. One of the objects of my invention is to provide improved means for surface-treating wood by which the cost of the finished wood product can be materially reduced through lessening the number of operations required to produce a satisfactory finish on the article, while another object of my invention is reducing the time required to produce a satisfactory permanent finish on wood surfaces. Still another object of my invention is to provide means by which the appearance of the treated wood surface is permanently improved, and the resistance of the treated wood surface to atmospheric and other agencies is permanently increased.

I have discovered that certain liquid chemical agents such as dilute acid and dilute alkali alone or in buffered solutions are readily taken up by smooth or planed surfaces of wood, and that such reagents exert a remarkable selective swelling action on the bundles of fibres which form the xylem or wood, having little or no action on the more compact or denser fibre groups, but exerting a very marked swelling action on the less dense and more porous fibre groups or aggregates. By moistening the surface of a smooth surface of wood with a suitable reagent having a pH value either higher or lower than that of pure water, or having high osmotic pressure as compared with water, this swelling effect occurs. Water produces a slight differential swelling effect upon some woods that are not entirely neutral in pH value, but is without effect upon other woods, and particularly wood of neutral pH and all the harder woods that are of principal value in cabinet making. All acids, both organic and inorganic, and all alkalies, both fixed and volatile, show a differential swelling effect, although in different measure. I find that dilute solutions of formic, acetic, propionic, butyric, citric, tartaric, hydrochloric, sulfuric, nitric, trichloracetic, malic, boric, sulfurous, oxalic and many other acids produce this characteristic effect, and the great number of acids which show this swelling effect is best explained by the theory that the action is due to osmotic pressure produced by a pH value sufficiently different from the normal relatively neutral condition of the wood to cause the observed swelling of the colloidal matter forming the cells which make up the softer portion of the wood. Just as all acids produce a selective swelling of the softer groups of wood fibres as compared with the harder groups of wood fibres, so all alkalies,

including ammonium hydroxide, and many acid and basic salts, produce a similar swelling. As some reagents color or otherwise harm the wood, I prefer to use certain specific reagents, and particularly a solution containing from 2% to 10% of acetic acid and from 2% to 10% of citric acid. I am fully aware, however, that the swelling which I have observed may be produced by a wide variety of reagents, including all water soluble acids and all water soluble alkalies, and a great number of salts, particularly the ammonium and alkali salts of formic, acetic, citric and tartaric acids, and the alkali and ammonium salts of sulfurous, thiosulfuric and hyposulfurous acids. The observed swelling is not confined to these specific reagents, however, and satisfactory swelling may also be obtained from 2% to 30% aqueous solutions of stannous chloride, zinc chloride, sodium potassium tartrate, and many other like water-soluble salts of relatively low molecular weight.

In the preferred practice of my invention I employ concentrations of my reagent varying from 5% to 15%, but my preferred reagent is a solution containing 5% of acetic acid and 5% of citric acid. I apply my reagent to the smooth, planed or sand-ed surface of the wood by means of a spray gun, or by a brush, or by dipping the wood in the reagent, or in any other convenient way, and I then allow a period of from one-half hour to five or six hours to elapse, within which the selective swelling of the softer fibre groups occurs.

When the softer fibre groups have reached a condition of maximum swelling the reagent begins to dry, but for some reason unknown to me the selective swelling of the fibre groups is not reversible, and the treated wood retains even after complete drying the roughened surface which resulted from the selective swelling of the softer fibre groups. I next subject the surface of the wood, roughened in the manner described by the selective swelling of the more porous and softer fibre aggregate groups, to an operation which has as its purpose the removal by tearing, cutting or abrasion of all portions of the wood which are swollen beyond the original plane represented by the original surface of the wood. This resurfacing operation can be conveniently performed by rubbing the surface of the treated wood with sand paper, emery paper, pumice stone, rotten stone or with any other satisfactory abrading or smoothing means, the object of the treatment being to completely remove by cutting or abrasion all the portions of the wood fibres which now stand out beyond the original smooth surface of the wood.

The result of this treatment is to leave a

smooth surface of wood made up in part of the original unswollen groups of dense fibre aggregates, and made up in part of the swollen and expanded remnants of the original fibre groups 5 of low density. One characteristic result of my treatment is that, instead of increasing the density of the softer groups of fibre elements, or of decreasing the density of the harder groups of fibre elements, I leave the harder and denser groups of fibre elements substantially unchanged, while I soften, swell and then remove part of the softer and more porous groups of fibre elements, and as a consequence the wood which 10 has been treated by my process shows a greater difference between its harder and its softer fibre elements than were shown before the treatment 15 was applied.

I next apply to the entire surface of my treated wood a protecting coating of an indurating 20 compound, that is capable of selectively penetrating the surfacial fibre groups. As a result of the effect of the preceding treatments as described, this indurating reagent will be absorbed in the least quantity by the originally dense or 25 compact fibre groups, and it will be absorbed in much greater measure, or in much greater quantity, by the softer and more porous remaining portions of the originally softer and less dense or less compact fibre groups. An ordinary alcoholic 30 solution of shellac forms a desirable indurating reagent, the shellac being left within the cells of the wood after evaporation of the solvent, or an aqueous solution of shellac in ammonia water or borax may be used. Varnish, 35 and particularly lacquer varnishes containing natural or synthetic shellac substitutes or natural resins, resinoids or resin substitutes may be employed, a very wide variety of indurating reagents being entirely suitable to the practice of 40 my invention, and the choice of a suitable indurating agent, either primary or secondary, being largely determined by the purpose for which the wood is to be used whether indoor or outdoor, and if outdoor, the degree of resistance 45 to atmospheric agents which is desired. I may, for example, treat the wood with an indurating agent and subsequently alter this indurating agent by heat or by the action of a chemical agent, for the purpose of further hardening the 50 indurating agent. I have even found that such indurating agents as aqueous solutions of natural gums, and particularly aqueous solutions of acacia, tragacanth and the like may be employed, although alkaline or alcoholic solutions of shellac, 55 rosin, resins and synthetic resins form the most satisfactory indurating agents.

Summarizing the treatment described, I first soften and swell the softer and less resistant fibre groups, without correspondingly softening 60 or swelling the harder, denser and more resistant fibre groups. I next abrade and remove the softened and swollen upper portions of the initially softer and less dense fibre groups, without correspondingly removing any portion of the harder and denser fibre groups, and I finally apply an indurating agent which is selectively absorbed by the initially softer and selectively softened and swollen fibre groups, without such reagent being equally absorbed by the denser 65 or less porous fibre groups, and as a final result of my process I obtain a surface which is equally hard and resistant over its entire area, through the indurating effect being much greater in the initially softer and subsequently further softened 70 portions than it was in the initially harder and 75

subsequently unaltered fibre aggregates made up of the denser, more compact and more resistant fibre groups.

To enable this method to be better understood, the drawing attempts to illustrate the effects 5 produced, at successive stages in the treatment of a piece of wood by my process.

Figure 1 is an enlarged transverse section through a piece of wood, cut in a direction perpendicular to the direction of the fibre groups 10 making up such piece of wood. *aaa* represents the upper surface portion of the harder, denser and more resistant fibre groups, while *bbb* represents the upper surface portion of the softer, more porous and less dense and less resistant fibre 15 groups and aggregates.

Figure 2 is a similar transverse section through the same piece of wood represented by Figure 1, after the upper or surface portions of the softer, more porous, less dense and less resistant fibre 20 groups have been swollen as shown at *ccc* by the action of a swelling agent as described. Figure 3 is a similar transverse section through the piece of wood represented by Figure 1 and Figure 2, after the raised portions of the softer fibre 25 groups *ccc* have been removed by cutting or abrasion, to leave the still less dense and more porous surface portions *ddd*. Figure 4 is a similar transverse section through the piece of wood represented by Figures 1, 2 and 3, after an in- 30 durating agent has penetrated into the softer fibre groups to varying extents and varying depths determined by the porosity of the fibre groups that has been caused or induced as a result of the treatment described. 35

It will be evident that the wood, treated as described, may subsequently be covered by any desired type of protecting film, such as paint, varnish, lacquer or the like. Very extensive tests have proven that wood, treated as described, offers greater resistance to both atmospheric agencies and mechanical wear, than wood treated by the usual finishing processes. Where stains are applied to the woods, a materially increased contrast effect is produced, due to the greater absorption of the stain in the softened fibre groups, the stain being preferably applied after the removal of the upper swollen portions of the fibre groups, and before the application of the indurating reagent. 50

My invention may be applied with substantially equal success to all of the customary types of hard and soft woods used in cabinet making and for like purposes. Although my invention is of maximum usefulness in the case of woods which 55 show the greatest contrast between the softer fibre groups and the harder fibre groups, my invention may be applied to all woods with some benefit, since I have found that in every wood there are differences in the hardness and density 60 of some of the longitudinal or transverse fibre groups as compared with other fibre groups, and the effect of my invention is to improve the surface strength of wood by rendering uniform the strength of the fibre groups which make up the 65 surface, by preferentially strengthening or indurating the softer fibre groups as compared with the initially harder or denser fibre groups in the manner described.

It will be noted that the effect of the swelling 70 reagent which I use is essentially to expand and swell the softer and more porous fibre groups or aggregates of the wood, without correspondingly softening and swelling the denser fibre groups or aggregates of the wood. The swelling is not in- 75

versely proportional to the density of the wood, however, as I find that dense fibre groups do not swell at all, or swell to so slight an extent as to be unnoticeable, while very porous fibre groups or aggregates expand and swell quite disproportionately to their relative densities. My process removes all of the expanded fibre groups that extend beyond the original plane of the wood, but I do not remove those portions of the fibre groups which, in their expanded condition, lie beneath the original plane of the wood. In my indurating step, I find that my indurating fluid is taken up by the expanded fibre group aggregates to a greater extent the lower the density of the fibre aggregates, but this proportionality is not a direct relationship, and the highly swollen and highly expanded fibre groups or aggregates take up an even greater quantity of the indurating fluid than would be represented by the proportionality of the densities of the fibre groups. As a result of this peculiar distribution of expansion or swelling, and of the absorption of the indurating fluid, I obtain as my final product a remarkable uniformity in the hardness of the fibre groups or aggregates, which is quite different from any effect ever obtained or described in the prior art.

If desired, I may prolong the action of my chemical swelling agent, in the first stage of my process, either by repeated applications of the swelling reagent, or by applying dampened cloth or damp paper, or wet sand over the surface, or by otherwise modifying the humidity of the air in contact with the surface that has been treated. In general I find, however, that when I use a dilute solution of acetic acid, or preferably a dilute solution of acetic acid and citric acid, a single application of the reagent produces entirely satisfactory swelling action, and no special control of humidity in the treating room is necessary.

When swelling agents are used which discolor the wood, or which have any other harmful effect upon the wood, I may, after the swelling treatment and after the following abrading treatment, remove or neutralize the swelling agent. I find that washing with water sufficiently removes most solutions of acid and basic salts which otherwise have a satisfactory swelling action, and alkali hydroxide, and any reagent which might produce an efflorescence from contact with the air, may be chemically neutralized or may be removed from the wood by washing. I am mentioning these possibilities for the purpose of making a complete disclosure, but in the application of my invention I find that the simplest treatment is the best, and a solution of from 2% to 10% of a volatile acid and particularly of acetic acid, with from 2% to 10% of a solid acid such as citric acid, tartaric acid, or a mixture of two volatile acids such as acetic acid and trichloroacetic acid, gives such extremely satisfactory results that it is not necessary or desirable to employ other materials such as sulfuric acid, for example, which may in time cause some harmful action on the wood, or to employ solutions or salts that might in time have a damaging effect upon either the wood itself or on the overlying protecting films of paint or varnish which may be later applied.

In view of the very wide choice of indurating agents which I may employ, broadly comprising any satisfactory solid natural or synthetic resin or resin-like substance, it is undesirable to name a wide variety of materials, and I find that ordinary shellac is an almost ideal indurating agent for my purpose, although many other natural and synthetic resins may be employed, particularly in

connection with very hard woods, where a very hard indurating agent is necessary to equal the hardness of the harder fibre groups. It will of course be evident that my indurating agent may be further hardened if desirable by suitable heat treatment, and this is particularly effective when using some of the newer synthetic resins which polymerize spontaneously with time, or under the influence of very mild heat, to form extremely effective penetrants and indurants for the softened and expanded fibre groups treated in accordance with my invention.

It will be evident that many changes may be made in the process as described without departing from the essential principles of my invention as herein described, and accordingly no limitations should be placed upon my invention except as indicated in the appended claims.

I claim:

1. The process of treating wood which comprises exposing a smooth surface of wood to a selective swelling reagent to swell the softer fibre groups to a greater extent than the harder fibre groups, restoring a smooth surface to the wood by removing all portions of the swollen fibre groups which extend beyond the original plane surface of the wood and selectively filling the fibres at the surface of the wood with an indurating material which penetrates the softer swollen fibre groups more readily than the initially harder and subsequently unchanged fibre groups.

2. The process of treating wood which comprises exposing a smooth surface of wood to a selective swelling agent comprising an acid to swell the softer fibre groups to a greater extent than the harder fibre groups, restoring a smooth surface to the wood by removing all portions of the swollen fibre groups which extend beyond the original plane surface of the wood and selectively filling the fibres at the surface of the wood with a resinous indurating material which penetrates the softer swollen fibre groups more readily than the initially harder and subsequently unchanged fibre groups.

3. The process of treating wood which comprises exposing a smooth surface of wood to a selective swelling agent comprising a volatile acid to swell the softer fibre groups to a greater extent than the harder fibre groups, restoring a smooth surface to the wood by removing all portions of the swollen fibre groups which extend beyond the original plane surface of the wood and selectively filling the fibres at the surface of the wood with a resinous indurating material which penetrates the softer swollen fibre groups more readily than the initially harder and subsequently unchanged fibre groups.

4. The process of treating wood which comprises exposing a smooth surface of wood to a reagent having a pH value sufficiently different from the pH value of the wood being treated to induce swelling of the softer fibre groups present in the wood, restoring a smooth surface to the wood by removing all portions of the swollen fibre groups which extend beyond the original plane surface of the wood and thereafter selectively indurating the remaining portions of the swollen fibre groups at the surface of the wood by treatment with a resinous impregnating agent.

5. The process of treating wood which comprises exposing a smooth surface of wood to a selective swelling agent comprising a volatile acid and a non-volatile acid to swell the softer fibre groups to a greater extent than the harder fibre groups, restoring a smooth surface to the wood by

removing all portions of the swollen fibre groups which extend beyond the original plane surface of the wood and selectively filling the fibres at the surface of the wood with a resinous indurating material which penetrates the softer swollen fibre groups more readily than the intially harder and subsequently unchanged fibre groups.

6. The process of treating wood which comprises exposing a smooth surface of wood to a selective swelling agent comprising a plurality of acid substances to swell the softer fibre groups to a greater extent than the harder fibre groups, restoring a smooth surface to the wood by removing all portions of the swollen fibre groups which extend beyond the original plane surface of the wood and selectively filling the fibres at the surface of the wood with a resinous indurating material comprising shellac which penetrates the softer swollen fibre groups more readily than the initially harder and subsequently unchanged fibre groups.

7. The process of treating a smooth surface of wood which comprises decreasing the density of the fibre groups of lower density on such surface, without correspondingly changing the density of the fibre groups of higher density by means of a chemical swelling agent, removing a portion of the fibre groups of lower density projecting beyond the original surface without removing a corresponding part of the fibre groups of higher density, and impregnating the fibre groups of lower density with an indurating agent without correspondingly impregnating the fibre groups of higher density.

8. The process of treating a smooth surface of wood which comprises applying a chemical swelling agent to decrease the density of the fibre

groups of lower density on such surface without correspondingly changing the density of the fibre groups of higher density, removing a portion of the fibre groups of lower density projecting beyond the original surface without removing a corresponding part of the fibre groups of higher density, and impregnating the fibre groups of lower density with a solid indurating agent without correspondingly impregnating the fibre groups of higher density.

9. The process of treating wood which comprises exposing a smooth surface of wood to a selective swelling reagent to swell the softer fibre groups to a greater extent than the harder fiber groups, restoring a smooth surface to the wood by removing all portions of the swollen fiber groups which extend beyond the original plane surface of the wood and selectively filling the fibers at the surface of the wood with a finishing protecting material which penetrates the softer swollen fiber groups more readily than the initially harder and subsequently unchanged fiber groups.

10. The process of treating wood which comprises exposing a smooth surface of wood to a reagent having a pH value sufficiently different from the pH value of the wood being treated to induce swelling of the softer fiber groups present in the wood, restoring a smooth surface to the wood by removing all portions of the swollen fiber groups which extend beyond the original plane surface of the wood and thereafter selectively impregnating the remaining portions of the swollen fiber groups at the surface of the wood by treatment with a finishing protecting agent.

MARJORIE G. SNELLING.